

E. KUHN,

PROCESS FOR THE MANUFACTURE OF MERCURY OXID.

APPLICATION FILED JAN. 30, 1919.

1,299,581.

Patented Apr. 8, 1919.



INVENTOR:

EMIL KUHN

BY: *Frank DeGraaf*

ATTORNEY.

# UNITED STATES PATENT OFFICE.

EMIL KUHN, OF BASEL, SWITZERLAND.

## PROCESS FOR THE MANUFACTURE OF MERCURY OXID.

Specification of Letters Patent.

Patented Apr. 8, 1919.

1,299,581.

Application filed January 30, 1919. Serial No. 274,083.

To all whom it may concern:

Be it known that I, Dr. EMIL KUHN, a citizen of the Swiss Republic, and resident of Basel, Switzerland, have invented a new and useful Process for the Manufacture of Mercury Oxid, of which the following is a full, clear, and exact specification.

Heretofore the preparation of mercury oxid was obtained by electrolyzing alkaline solutions with mercury anode or by dissolving metallic mercury in acids and precipitating the mercury oxid from the solution obtained by means of alkalis or by the combustion of mercury with air or oxygen.

15 The two first processes have the inconvenience that owing to the solubility of the mercury oxid in water, which is not to be neglected, losses occur which can only be avoided partly by complicated provisions.

20 These losses are also increased by the facts that the intermediary products must be subjected to various manipulations, as propulsions, precipitations, out-washings and the like.

25 The oxidation of mercury by oxygen begins at temperatures above 300° C., but proceeds then very slowly. At higher temperatures, the oxygen pressure of mercury oxid is already perceptible, as it is shown by the 30 equilibrium essays of P. Laban (*Comptes-Rendus* 1899, vol. 128, page 825); therefore the oxidation cannot be complete in this latter case. But for the technical manufacture of mercury oxid the slow formation 35 at low temperatures is equally disadvantageous as the incomplete union of mercury and oxygen at higher temperatures, setting aside the other inconveniences inherent to every process working with mercury vapor.

40 The following process is also based on an oxidation of metallic mercury by gases containing oxygen, but is distinguished hereby that the oxidation by gases containing oxygen is effected with the aid of dry nitrogen 45 oxids acting as oxygen transmitters.

The advantages of the process are the following:

The attack of the metallic mercury occurs at a temperature, at which its vapor pressure 50 is still very small, for instance at ordinary room temperature. Secondly the reaction mass can remain in a closed vessel during the whole process, that is to say until the metallic mercury is transformed into the 55 achieved dust-fine oxid, so that all mercury losses are excluded. Thereby the necessary apparatus has only to be some greater than

the dimension requested by the volume of the oxid produced in an operation, so that the transformation of very large quantities 60 can be effected in a small room easy to control. Fourthly no other materials than mercury and oxygen are employed and fifthly the apparatus can be formed by iron in opposition to the working with aqueous nitric 65 acid.

The drawing illustrates a simple form of apparatus for performing the process.

Example: Mercury is instilled, by drops, in the iron vessel 1 of the apparatus represented by a partly sectional elevation in the accompanying drawing, filled about to the middle with liquid  $N_2O_4$ , while oxygen or air is introduced simultaneously in the vessel.

70 The attack of the mercury occurs according to the following formula:



The vessel is provided with a reflux cooler, in order to let drop retrograde the  $N_2O_4$ , 80 vaporized by the reaction heat. Obviously the mercury can be placed in the vessel and the  $N_2O_4$  introduced by drops in the latter. After complete transformation of the mercury into nitrate, the reflux cooler is set out 85 of service and the excess of  $N_2O_4$  remaining in the vessel 1 driven over in a similar vessel 2. Hereafter the content of the vessel 1 is heated, preferably while stirring slowly, whereby the mercury nitrate is decomposed 90 according to the formula



The  $NO_2$  evolved in the vessel 1 is collected as  $N_2O_4$  in the second vessel 2. The 95  $HgO$  obtained is dustfine, needs consequently no grinding and is furthermore very pure. Then the vessel 1 is replaced by another or its  $HgO$  is discharged therefrom and the same process is repeated, the vessel 2 taking 100 up now the functions of the vessel 1 vessel 1 now serving to receive the  $NO_2$  expelled from vessel 2. One can obviously also proceed in the manner, that the  $N_2O_4$  collected in the vessel 1, by means of compressed air 105 and mercury is again instilled by drops in the vessel 1, etc. The process does not change, if the supply of oxygen is, in the course of the decomposition, intentionally or accidentally insufficient for the quantitative retroformation of  $NO_2$ ;  $NO$  is then formed, which dissolves in the  $N_2O_4$  contained in the vessel 110 2, forming  $N_2O_3$  which can also be oxidized easily to  $N_2O_4$  by introducing oxygen, as

well before as during the treatment of a fresh quantity of mercury.

When oxygen is employed for the oxidation there exists theoretically no sources of losses neither for Hg nor for nitrogen oxid. In this manner with a very small quantity of  $N_2O_4$  technically very large quantities of mercury can be combined with oxygen, without any consumption of essential quantities of the auxiliary body and without any manipulation of the intermediary products outward of the apparatus. The  $N_2O_4$  acts only as oxygen transmitter.

A special advantage of this process consists in the possibility of its application for the transformation into mercury oxid of mercury wastes as they result for instance

from the synthesis of organic bodies from acetylene.

What I claim is:

The herein described process for the manufacture of mercury oxid by oxidation of metallic mercury, wherein the oxidation by gases containing oxygen is effected with the aid of dry nitrogen oxids acting as oxygen transmitters.

In witness whereof I have hereunto signed my name this 2d day of December, 1918, in the presence of two subscribing witnesses.

DR. EMIL KUHN.

Witnesses:

H. H. DICK,  
ARNAUD RITTER.